

Jan. 22, 1929.

1,699,612

H. DOAT

METHOD FOR THE PRODUCTION OF UNHARDENED CASTINGS IN METAL MOLDS

Filed Oct. 26, 1925

Fig. 1



Fig 2



Inventor:

Henri Doat

By *Lucie Doat*  
Attorney

## UNITED STATES PATENT OFFICE.

HENRI DOAT, OF BRUSSELS, BELGIUM, ASSIGNOR TO COMPAGNIE GENERALE DES CONDUITES D'EAU, SOCIETE ANONYME, OF LIEGE, BELGIUM.

## METHOD FOR THE PRODUCTION OF UNHARDEDENED CASTINGS IN METAL MOLDS.

Application filed October 26, 1925, Serial No. 64,879, and in Belgium November 4, 1924.

This invention relates to the production of unhardened castings in metal molds.

It is known, in connection with making iron castings, that the sudden contact of the molten metal with the metal sides of the mold causes an outer layer of white cast iron to form on the surface of the casting. In order to prevent this phenomenon it is usual to provide the mold with a lining which prevents the cooling from taking place so rapidly as to lead to the formation of such outer layer of white cast iron.

The present invention is specially directed to the production of unhardened castings by making use of a lining material which also presents additional advantages.

Said lining acts not only as a means of protection for the mold itself and for preventing a too rapid cooling of the metal remaining in contact therewith during the casting process, but also serves a physico-chemical function which co-operates with those just mentioned in causing the formation of a superficial layer of grey cast iron on the casting, said layer being characterized by flakes of graphite without any large excess of cementite.

According to the invention, said lining is composed of silicon, or of an alloy or substance containing silicon in the free state, in combination or in solution.

According to one method of carrying out the invention in a particularly advantageous manner from the point of view of the cost of production, said lining may be composed of ferro-silicon.

In the case of iron castings, the physico-chemical phenomena taking place result in increasing the tendency of the iron carbide to decompose in such a way that, in spite of the high rate of cooling of the outer layer, the  $Fe_3C$  therein is reduced to its elements and therefore furnishes a grey cast iron characterized by flakes of graphite without any large excess of cementite, in place of a white cast iron with cementite in large excess.

This method offers therefore the two-fold advantage of facilitating the formation of grey cast iron on the surface of the casting (that is to say, preventing superficial hardening) and, on the other hand, of considerably prolonging the working life of the metal mold.

When applied to the metal molds used for making pipes and pillar by centrifugal cast-

ing, the invention provides for the distribution of the ferro-silicon, or the substance or alloy mentioned above, over the interior surface of the mold by the action of the centrifugal force.

With this object, these materials may be introduced into the mold, which rotates on an approximately horizontal axis, said introduction being effected either by means of a trough extending all along the mold or by means of a charging nozzle. In the latter case a relative longitudinal movement is imparted to the rotary mold and said nozzle.

In order to turn out the maximum number of castings in a given time, and especially the largest number of pipes in the case of a rotary cylindrical mold, the invention also provides for the introduction and centrifugal distribution of the said lining material just prior to the introduction of the molten metal.

In the case of molds having a large inner surface, these successive introductions may be effected on portions of said surface and before the whole of the surface has been covered with the lining material.

The invention also provides for the restriction of the application of the lining material to certain parts only of the mold, the other parts being left bare or covered with a lining of different thickness from that on the first parts aforesaid.

Various details of the applications of the invention will now be given by way of example.

As already mentioned, the invention provides for the employment of silicon, or of an alloy or substance containing silicon, a preferred form being ferro-silicon. In this latter case a mixture containing 40 to 80% of silicon may be used, though, of course, in certain contingencies, the percentage of silicon may be outside these limits. In some cases, ferro-silicon may be replaced by a material containing a different product alloyed with silicon.

In some cases, use may also be made of pure silicon, which acts simultaneously as a chemical agent on the metal of the casting and as a protective agent on the mold itself.

The substance or alloy with a silicon base may be used either in the form of a paste, rendered adherent by means of a binding medium of any kind, or in the state of a more or less fine powder.

The material employed may be placed in position prior to each casting process in order

60

65

70

75

80

85

90

95

100

105

110

to repair the lining, a portion of which is worn away every time a casting is made.

A coating of adhesive paste may be prepared by mixing powdered ferro-silicon with 5 an adhesive substance, such as gluten, linseed oil, molasses, rosin, varnish, flour, dextrin or colophony. This coating may be applied, for example, by means of a brush, a vaporizer or an atomizer.

10 The mold may be heated to a certain temperature, or the material with a silicon base may be heated prior to its introduction into the mold.

15 The invention covers, of course, all bodies or compounds having an action similar to that exerted by silicon as set forth above.

20 In the particular application of the invention to molds intended for centrifugal casting, and where the material is used in the form of powder, the latter may be introduced into the mold by hand, either while the mold is stationary or rotating, if the mold is a short one.

25 In the case of a longer mold, such as is used, for example, in casting pipes, use may be made, for example, of one or the other of the devices illustrated in the accompanying drawings, wherein:—

30 Figure 1 is a perspective view, in partial section, of a typical rotary mold provided with a single trough for the distribution of the lining material.

35 Figure 2 is a cross section through a rotary mold provided with two troughs for the distribution of the lining material and molten metal respectively.

40 In the case of Figure 1, a trough 1 of approximately the same length as the mold 2, is adapted to slide on a guide rod 3 and to pivot on same so as to discharge, into the mold, the substance with a silicon base with which said trough is charged.

45 This substance is then distributed, by the centrifugal force, all over the sides of the mold, and when this has been done, the molten metal can be poured in.

50 It will be understood that the trough might be replaced by a nozzle discharging the said substance. In such case, in order to cover the sides of the mold all over, it will be neces-

sary to arrange for the production of a relative longitudinal movement, equivalent to the length of the mold, between the mold and the nozzle.

55 In order to ensure the quick succession of the operations of distributing the substance with a silicon base and the pouring of the molten metal, the invention provides for the arrangement, in the interior of the mold (see Fig. 2), of two guide rods 3, on which the trough 4 containing the silicious material and the trough 5 containing the molten metal are adapted to slide and tilt in succession, in the directions indicated by the arrows.

60 It will be understood that the two troughs may be interconnected and arranged in such a manner as both to tilt in the same direction, for example around the same axis, so that the successive distribution of the silicious material and the molten metal may be effected 70 automatically by a single actuating means.

65 It should be noted that the invention also provides for coating portions only of the mold with the silicious lining, leaving other portions bare or covering them with another kind of lining. In using a trough for the distribution of the silicious material, this result could be accomplished, for example, by providing the trough with lateral compartments, some being charged with the material, and others left empty. In the case of a nozzle, a cock controlling the delivery could 75 be provided.

#### What I claim is:

80 In a method of producing unhardened castings in rotating metal molds, the step of introducing into the mold, while it is rotating and prior to the introduction of the molten metal, a ferro-silicon alloy in the state of loose powder, the grains thereof being held 85 against the surface of the rotating mold by centrifugal force; said alloy forming a lining which protects the rotating mold during the casting operation and afterwards becomes incorporated chemically in the outer portion 90 of the casting to convert the white cast metal into gray cast metal characterized by flakes of graphite without large excess of cementite.

95 In testimony whereof I affix my signature.

HENRI DOAT.